

Feb. 24, 1931.

F. M. DORSEY

1,793,914

APPARATUS FOR TREATING FLEXIBLE METAL BODIES

Filed Sept. 2, 1927



Fig. 2



Fig. 3



Fig. 4



Fig. 5



Inventor  
Frank M. Dorsey  
By his Attorney  
Edward M. Evans

## UNITED STATES PATENT OFFICE

FRANK M. DORSEY, OF SOUTH EUCLID, OHIO, ASSIGNOR TO MADSENELL CORPORATION, OF PORTSMOUTH, OHIO, A CORPORATION OF NEW YORK

## APPARATUS FOR TREATING FLEXIBLE METAL BODIES

Application filed September 2, 1927. Serial No. 217,260.

My present invention relates to apparatus for treating metallic bodies, particularly relatively elongated and relatively flexible metallic bodies, such as wires, ribbons, strips and the like, especially but not exclusively such bodies as are made of ferrous metals, such as iron or steel, which ordinarily contain surface carbon, superficially occluded gases, particularly hydrogen as a result of the usual acid pickling operations, lubricants, grease and other impurities, and aims to devise apparatus of the general character specified which is simple in construction, which is easy, convenient and economical to operate, and which enables the surface portions of such bodies to be efficiently and thoroughly cleaned and prepared for subsequent coating and other uses, especially for coating by electrolytic means. Other objects and advantages of the apparatus of the present invention will in part be pointed out in detail hereinafter and will in part be obvious to those skilled in the art to which the present invention relates.

In the accompanying specification I shall describe, and in the annexed drawing show, an illustrative embodiment of the present invention. It is, however, to be clearly understood that my invention is not limited to the specific embodiment thereof herein shown and described for purposes of illustration only. In connection with the foregoing illustrative embodiment of the apparatus of the present invention, I shall describe one form of method which may be practised in such apparatus. It is, however, to be clearly understood that such method forms no part of the present invention, being more fully described and being fully claimed in a co-pending application of mine filed of even date herewith and entitled "Methods of treating flexible metallic bodies."

Referring to the drawing, wherein I have illustrated the aforesaid illustrative embodiment of the present invention:

Fig. 1 is a view in longitudinal section more or less diagrammatically illustrating said embodiment;

Fig. 2 is a cross-sectional view of one form of metallic body, such as a wire, at one stage

of its manipulation in the embodiment of apparatus illustrated in Fig. 1 of the drawing;

Fig. 3 is a cross-sectional view of such body at another stage of its manipulation;

Fig. 4 is a cross-sectional view of such body at still another stage of its manipulation;

Fig. 5 is a cross-sectional view of such body at still a further stage of its manipulation.

Before describing the aforesaid illustrative embodiment of the present invention in detail, it may be desirable briefly to point out certain disadvantages and shortcomings of the field to which the present invention belongs. In this connection, I shall describe the invention as applied more particularly to the treatment of wire, although similar considerations apply in using the apparatus of the present invention in connection with other flexible metallic bodies, such as strips, ribbons and the like. Hitherto, in the manufacture of wire, it has been customary, as is well known to those skilled in the art to which the present invention relates, to start with an ingot which is shaped into a rod which is then drawn down to a wire with the use of a lubricant which often contains graphite or other solid lubricating material. In drawing the rod down to the wire, the lubricant is worked into the surface of the wire and is also baked into the surface by the annealing treatments, to which the rod and wire are generally subjected to keep the same workable for the subsequent drawing operations.

As a result of these manipulations, by the time the rod has been worked down to a wire of the desired diameter, the carbonaceous impurities will be found to have been worked into the surface of the wire to such an extent that their removal is a difficult matter. In fact, various types of apparatus and various types of chemical and mechanical treatments have hitherto been employed with only partial success for this purpose. The impurities are obviously undesirable since they often render the wire brittle and since they render the subsequent coating liable to become readily separated, especially if the wire, as is often required, has to be bent in use.

These disadvantages and shortcomings of the prior art are readily overcome by means of the apparatus of the present invention. Referring to the drawing, wherein the aforesaid illustrative embodiment of the present invention is more or less diagrammatically illustrated, 10 indicates a metallic body, preferably relatively elongated, and preferably relatively flexible, such as a wire in the form of a coil of wire 11 wound up on the drum 12. The wire 10 may be made of steel, iron or other ferrous metal, which generally contains carbon and occluded gases at its surface, or may consist of wire made of copper, bronze or brass or other copper-containing metal which generally contains occluded hydrogen and other gases adjacent its surface, in addition to the graphite or other lubricant which has been worked into the surface portions of the wire or other flexible metallic body during the drawing or equivalent operations.

13 is a take-up drum, which takes up the treated wire or the like. The drums 12 and 13 are preferably insulated from each other and from the wire 10, as by being made of insulated material or by having an outer layer or sheath of insulating material applied thereto. It may here be stated that the drums 12 and 13 may be actuated by any suitable mechanism, not here deemed necessary to be shown, at a predetermined rate of speed, to permit the treating operation to be efficiently conducted.

20 indicates a container, which may be in the form of a vat, preferably one lined with lead or other material which will protect the vat from the cleaning means intended to be contained therein. 30 indicates means for flexing the wire or other metallic body a predetermined number of times, preferably in different or opposite directions and preferably about different flexing axes so as to more fully expose the impurities contained at surface portions of the wire or other flexible metallic body, in order to permit the cleaning operation to be more effectively carried out. Preferably the flexing means 30 comprises a plurality of flexing members 31. I prefer that the flexing members 31 shall be arranged in two series generally designated by reference characters 32 and 33, respectively. The flexing members 31 preferably comprise rolls or rollers over which the wire may be readily passed in its travel from the unwinding drum 12 to the take-up drum 13, the diameter of the rollers 31 being preferably such as not to subject the wire 10 to too sharp a bend. In fact, the diameter of the drum 12 should be so chosen as to flex the wire just enough to open up enough of the surface portions of the wire adjacent the flexed portions to permit the cleaning operation to be effectively conducted, and no more.

35 The wire 10 passes under the series 33 of

rollers 31 and over the series 30 of such rollers. 21 indicates a bath of sulphuric acid preferably of a strength of more than about 55° Beaumé, as of a strength of about 66° Beaumé, preferably ordinary commercial concentrated sulphuric acid. The wire 10 preferably serves as an anode, for which purpose I connect the wire at the points 40 and 41 with the positive poles of a suitable source of direct current, at, for example, a voltage of about 12 volts, although voltages higher than that, as, for example, 20, 25 or 30 volts may be employed. The bath 21 is preferably maintained at a temperature of about 100° F. by any suitable means, such as a hot water coil 22. If the bath shows a tendency to become overheated, cold water may be passed through the coil 22 in order to maintain the bath at the desired temperature. For cathodes, I may employ the strips or plates 42 interposed between the folds or bends of the wire 10. These cathodes may be suitably connected to the negative pole of the source of current, not here deemed necessary to be shown, to the positive pole of which the portions of the wire 10 are connected adjacent the poles 40 and 41.

I also provide means for turning the wire or other metallic body 10 so that during the flexing operation, the body will be flexed about different axes so that all of the surrounding surface portions of the same will have their texture more or less opened up for the cleaning operation. The turning means, generally designated by reference character 50, may comprise a clamp having the handle 51 and being so arranged that the wire can be turned through any desired angle, first in one direction and then in the opposite direction, so that the wire will not be subjected to too great a torsional force.

For example, and referring more particularly to Figs. 2, 3, 4 and 5 of the drawing, the wire will be shown to have been divided into four quadrants designated 1, 2, 3 and 4 respectively. The arrow in each case indicates that quadrant which is outermost when the wire is flexed and the surface portions of which will therefore be opened to permit the cleaning operation to be conducted. In Fig. 2, the quadrant 1 has the surface portions of the same so opened up for the cleaning operation. In Fig. 3, which corresponds to the return of the flexed wire, the quadrant 3 has its surface portions so opened. In Fig. 4, the wire has been turned through about 90° by the turning means 50 and thus the quadrant 2 has its surface portions so exposed, while in Fig. 5 the opposite quadrant, namely quadrant 4, has been flexed and has its surface portions so exposed.

It may here be stated that the cathodes 42 may comprise sheets of iron or steel, or of lead, or of iron or steel coated with lead. It may here also be stated that the cathodes

may be mounted and connected in any suitable manner. It may here further be stated that the level 21' of the electrolyte 21 in the vat 20 may be and preferably is maintained at such a point that the upper ends of the loops 5 of wire passing over the upper series 32 of rollers 31 will be above the level of the electrolyte so that the upper turns of the wire 10 will be successively exposed to the air to assist the degasifying action.

In operation, that portion of the wire 10 between the positive poles 40 and 41 acts as an anode, the strips 42, which are preferably equidistantly spaced between the turns of 15 wire 10, acting as cathodes in the bath of strong or concentrated sulphuric acid. While a considerable cleaning action will be effected in those portions of the wire 10 between the series 32 and 33 of flexing members 31, greater cleaning action per unit of 20 length of wire will be effected at the portions of the wire which are momentarily flexed by the members 31 and the outer surface portions of which are therefore opened up so 25 as to facilitate the cleaning operation.

The cleaning action is such as to remove to a great extent, if not entirely occluded hydrogen and other gases, also carbon, lubricant and other impurities present adjacent the 30 surface portions of the treated body. The current density, which may be any desired amount but which is preferably from about 30 to about 50 amperes per square foot of treated surface, is at a maximum adjacent 35 the pole 40 and at a minimum the pole 41, being at a mean or average value adjacent the middle point of the wire 10. This current density will be found to attain a mean or average and substantially fixed value after 40 the treatment is under way, substantially fixed for a particular speed of operation and for a particular type of wire, varying for wire of different types and for different speeds of travel. As already stated, the voltage 45 of the direct current employed may be about 12 volts, although direct current of about 20, 25 or 30 volts may also be employed, the current being preferably direct current although a uni-directional, pulsating current 50 may be employed instead.

The treated wire may now be rinsed with water, which may, if desired, contain a slight amount of ammonia or other alkaline substance to neutralize the sulphuric acid used 55 in the cleaning treatment. The rinsing means, forming no part of the present invention, has not been deemed necessary to be shown here.

This completes the description of the afore- 60 said illustrative embodiment of the apparatus of the present invention. It will be noted that such apparatus is simple in construction, may be readily and economically fabricated and assembled, and is highly 65 efficient in operation for the intended pur-

pose. Other advantages and superiorities of the apparatus of the present invention will readily occur to those skilled in the art to which the present invention relates.

What I claim as my invention is as follows:

Apparatus for treating a flexible elongated metal body, which comprises a container, means associated with said container for successively flexing said body in different directions at predetermined surface portions of 70 the same more fully to expose impurities present in said body at said surface portions and means for turning said body about an axis at an angle to the axes of flexing of said body.

In testimony, whereof, I have signed my name to this specification this 15th day of 80 August, 1927.

FRANK M. DORSEY.

85

90

95

100

105

110

115

120

125

130